

# United States Patent [19]

Parent

[11] 3,958,990

[45] May 25, 1976

[54] TRANSFERRING TONER TO AN AMINE  
COATED SHEET

[75] Inventor: **Richard A. Parent**, Fairport, N.Y.

[73] Assignee: **Xerox Corporation**, Stamford,  
Conn.

[22] Filed: **Apr. 17, 1975**

[21] Appl. No.: **569,137**

## Related U.S. Application Data

[62] Division of Ser. No. 465,965, May 1, 1974.

[52] U.S. Cl..... **96/1.4; 96/1.2;**  
427/16; 427/24

[51] Int. Cl. <sup>2</sup>..... **G03G 13/16; G03G 13/22**

[58] Field of Search ..... **96/1.2, 1.4; 427/16,**  
427/24

## [56] References Cited

### UNITED STATES PATENTS

3,493,412 2/1970 Johnston et al..... 96/1.4 X  
3,535,112 10/1970 Dolce et al. .... 96/1.4

|           |         |                   |          |
|-----------|---------|-------------------|----------|
| 3,539,340 | 11/1970 | Dolce et al. .... | 96/1.4   |
| 3,539,341 | 11/1970 | Dolce et al. .... | 96/1.4   |
| 3,811,914 | 5/1974  | Saito et al. .... | 96/1.4 X |
| 3,847,642 | 11/1974 | Rhodes ....       | 96/1.4 X |
| 3,854,942 | 12/1974 | Akman ....        | 96/1.2   |
| 3,871,879 | 3/1975  | Arai....          | 96/1.2   |

Primary Examiner—**Roland E. Martin, Jr**

## [57] ABSTRACT

A transparency is disclosed, which is suitable for use in a multicolored xerographic reproduction process comprising a transparent, thermoplastic film sheet having at least one surface coated with a material selected from the group of nonvolatile amine compounds. The coated transparency, when used in a multicolored electrostatic copying process improves adhesion of the multicolored image thereon and permits reproduction of colors and color densities in said image which correspond well to the copied multicolored original.

**6 Claims, No Drawings**

## TRANSFERRING TONER TO AN AMINE COATED SHEET

This is a division of application Ser. No. 465,965, filed May 1, 1974.

### BACKGROUND OF THE INVENTION

This invention relates to xerographic reproduction and specifically to transparencies which are suitable for use in a xerographic reproduction process.

Transparencies are a highly useful product in visual education since an image on a transparency may be projected with the necessary degree of magnification onto a screen where it may be viewed by a large number of persons. Transparencies have heretofore been made by photographic reproduction of the desired image and accordingly have required the skill of an individual who is familiar with complex photographic reproduction processes. Photographic reproduction of transparencies also requires the expenditure of a large amount of time and money and is thus undesirable for this reason. Therefore, an easy and inexpensive means for the production of transparencies has been sought whereby transparencies could be conveniently and economically imaged and then used an unlimited number of times in visual education programs.

The advent of xerography and electrostatic copying as generally disclosed by Carlson in U.S. Pat. No. 2,297,691 has proven to be a highly successful process for reproduction with the inherent advantages of speed and reliability. In a usual xerographic process, an electrostatic image of an object is formed on a recording member such as a xerographic plate or drum. The xerographic plate may comprise a layer of photoconductive material, such as selenium on a conductive metal backing. The latent electrostatic image which is formed on the photoconductive material is developed into a powdered image which is then subsequently transferred to a sheet of paper and affixed thereon to form a permanent print.

The xerographic process has therefore proven to be an easy and reliable means for the production of transparencies. Transparencies made by a xerographic process are produced by forming an electrostatic image of the desired object, developing it, and then transferring it to a transparent sheet material with the image being permanently affixed or fused thereto by either the application of heat or by the action of a solvent vapor. In either case the toner which is used to develop the powdered image is coalesced on the sheet material by the fusing technique to form a permanent image thereon. Solvent fusion techniques, for transparent materials made by a xerographic process, for example, are illustrated in U.S. Pat. Nos. 3,049,810 and 3,148,078.

While the xerographic reproduction process is an apparent solution to the problem of economical and efficient production of transparencies, other problems have also been encountered with its use in the production of transparencies. One of the most pronounced problems with producing transparencies by an electrostatic copying process is to get the powdered or developed image to adhere well to a transparent film material before the image is permanently affixed thereto by fusing. Failure to achieve this results in an irregular substrate-toner interface resulting in extensive light scattering in projection and, therefore, loss in color. A further problem encountered is obtaining proper and

uniform density of the image after fixing or fusion and without resultant damage to the transparent film material either in the fusion process or in the transfer system employed within the machine. For this reason, various coating and combinations thereof with various types of transparent sheet materials have been previously proposed to obviate some of these difficulties. Included are various single component polymeric coatings such as are exemplified in U.S. Pat. Nos. 3,539,340; 3,539,341 and 3,535,112.

The above coatings, while of some assistance in improving adhesion of the developed electrostatic image to a transparent film material, nevertheless, are not entirely suitable when transparencies are produced by 15 a multicolored xerographic imaging process. The difficulties encountered with a multicolored imaging process and transparencies produced thereby are due in part to the multicomponent pigmented and dyed developers required in the multicolored imaging process and their varying degree of attraction for the transparent sheet material. Furthermore, the problem of getting the correct degree of coalescence of the toner particles in the permanent image is an even more critical matter with multicolored imaging than with single color image 25 development. This increased criticality is due to the fact that black or single color transparencies only require complete opaqueness or nonopaqueness to produce a transparency which has images suitable for projection.

30 Multicolored transparency images, on the other hand, must allow for a certain degree of color density for each color or color combination in the image which is sufficient and uniform enough to allow projection of a uniform and true color. This, therefore, requires a 35 different and unique combination of materials being employed and more critical controls being imposed upon the transparent materials which are used in a multicolor xerographic imaging process to obtain the correct degree of attraction of toner to the transparent sheet as well as proper coalescence of toner particles for consistent hue and good color density.

The instant invention relates to a transparency which fulfills all the requirements for use in the production of multicolored electrophotographic images. The subject 45 invention is particularly suited to overcome difficulties associated with the projection of color xerographic images which are formed on transparencies. In addition, the instant invention utilizes materials which are readily available and are relatively simple to work with. 50 By means of the subject invention effective transparencies for use in a xerographic color process are easily prepared.

It is an object of the present invention to provide a 55 transparency which is permanent in nature and having the sheet strength necessary to allow repeated use thereof for visual education purposes.

It is also an object of the present invention to provide for production of a color transparency by a xerographic multicolor imaging process which in turn eliminates the 60 skill of a technician who is trained in reproduction photographic processing.

These and other objects, as well as the scope, nature and utilization of this invention will be apparent by the following detailed description and appended claims.

### SUMMARY OF THE INVENTION

It has now been determined that the general objective of producing a transparency which will perma-

nently hold a true and consistent multicolor xerographic image may be best achieved by utilizing a transparent, thermoplastic, film sheet such as a polysulfone or polycarbonate sheet material, followed by the coating of this sheet prior to xerographic imaging with a nonvolatile amine compound such as 1,8-diamino octane, n-octadecyl amine, or n-dodecyl amine, among others. It is this coating composition which has been found to insure that all colored pigments required in the multicolored reproduction process are properly attracted to and held by the transparent sheets during imaging and sheet transfer so that a permanent image having uniform and accurate color densities may be then fused on the transparent sheet. This coating overcomes the previously noted difficulties with producing a transparency by a multicolored electrostatic copying process, among which are poor adherence of the developed xerographic image on the transparent film, as well as difficulty in insuring that a consistent and true color density is developed from the colored original which will also be suitable for projection or magnification on a screen. As indicated, these problems while existing with single color xerographic imaging, are even more pronounced when a multicolored xerographic process is employed.

#### DESCRIPTION OF THE PREFERRED EMBODIMENT

In the process of multicolored xerographic reproduction, a subtractive color to color reproduction technique is used to develop images formed on the photoconductive layer. Furthermore, a multicolor xerographic imaging process may also employ multiple scanning of the colored original at different wavelengths of light to produce multiple images corresponding to each primary color involved in the original. These primary color images may be then recombined to form a single multicolored image corresponding to the original by using a multicomponent or multicolored toner in a subtractive color to color reproduction process. A subtractive color to color reproduction process is illustrated in U.S. Pat. No. 3,057,720.

Toners which are employed in multicolor xerography use subtractive primary colors, yellow, cyan (blue green) and magenta. These in turn are used to reproduce a wide gamut of colors normally found in the colored original. For the purposes of illustration, when subtractive mixing of the yellow and cyan colorants take place, greens are obtained. Likewise, the mixing of magenta and yellow colorant in varying amounts reproduces reds, while combining the cyan with magenta results in the reproduction of blues. Mixtures of equal amounts of each toner, of course, will produce a black image.

Production of the multicolored copy from the colored original may be appropriately achieved by any multicolored xerographic imaging process. It is not intended that this invention be limited by particular variations in the multicolored xerographic imaging processes that might be employed or with the equipment used in said process. Nevertheless, for the purposes of illustration, a suitable process for color imaging begins with proper discernment of the color composition of the original subject matter and recording thereof. This may be conveniently accomplished by sequential optical scanning of the color original a number of times to formulate a sequence of the latent electrostatic images which correspond to the primary col-

ors in the original. This is accomplished by the light image passing through an appropriate color filter so that the latent image is then in effect, color separated according to the various primary colors. Theoretically, the latent image which is formed by passing the light image through a green filter should require the magentas (the complementary color) as areas of relatively high charge density on the drum surface, while the green (the separated color) should cause a low-charged density level. The magentas are then made visible by applying a green absorbing magenta toner to the image bearing member. By the same token, a blue separation is developed with a cyan toner. The three developed color separations are then brought together in registration upon the final sheet of support material to produce a multicolored facsimile of the original colored document copy.

It is this multicomponent developer system used in a subtractive color to color reproduction process which presents numerous problems when, for example, a color transparency is produced thereby which will reproduce, with uniform and accurate consistency the color densities which correspond to the colored original.

In the production of transparencies by a multicolored xerographic imaging process according to the present invention, a transparent, thermoplastic film sheet material is selected as the support material upon which the multicolored xerographic image is to be developed. Although the sheet material may be any suitable thermoplastic film material which has the clearness, strength and heat resistance to allow repeated projection thereof, materials which are particularly preferred for the present invention include thermoplastic resins such as the polysulfones, polycarbonates and polyesters.

Thermoplastic sheet material which may be conveniently utilized in the present invention includes polysulfone sheet material which are commercially available from Rowland Products Inc., Kensington, Conn. and Instar Supply Co., Inc. New York, N.Y. under the name Folacron PSN, as well as polycarbonate sheet materials commercially available from General Electric Corp., Waterford, N.Y. under the names LEXAN SL1007 (a tetrachloro-polycarbonate) and LEXAN DL616 (a tetrabromo polycarbonate). These materials may be selected from any thickness range desired, although in selecting film thickness, the films should be thick enough to have the necessary strength but still be thin enough to remain flexible throughout continuous use thereof. A suitable thickness of the film suitable for use in xerographic imaging, will generally be from about 3 to 8 mils.

The thermoplastic film material is then coated with an aliphatic amine coating composition which has been found to significantly improve adhesion of a multicolored xerographic image to a transparency during the xerographic development process while at the same time during image fusion, permitting accurate reproduction of color density on the transparency. The coating in this regard has been found to assist in permanent fixing or fusing of the developed image to the transparency by either solvent vapor or heat fusion techniques.

The coating developed herein comprises a mixture of a nonvolatile amine and a suitable solvent for coating purposes. The meaning of nonvolatile within the context of the present invention are those amines with

melting points above 40°C. Typical of amines within the purview of the present invention are:

primary amines



where R = linear or branched alkyl groups of from 10 to 30 carbon atoms.

secondary amines



where R and R' are linear or branched alkyl groups having from 10 to 30 carbon atoms.

tertiary amines



where R, R' and R'' are linear or branched alkyl groups of from 10 to 30 carbon atoms.

diamines



where n is from 2 to 10 and R, R'', R''', R'''' are linear or branched alkyl groups of from 10 to 30 carbon atoms.

While any and all of the above nonvolatile amines may be used within the purview of the present invention, especially preferred amines are 1,8-diamino octane, n-octadecyl amine, n-dodecyl amine, tallow amine, and hydrogenated tallow amine all supplied by the Armour Industrial Chemical Company of Chicago, Ill.

The coating mixture will be normally applied to the transparent film material in the form of a solution and because of this, the choice of solvents to provide the solution is important, relative to the coating composition, since it must not cloud or change the film material and it must at the same time provide enough solubility for the coating composition to provide a clear uniform coating on the transparency with no evidence of component insolubility.

Suitable solvents for the aliphatic amines are those organic liquids which will dissolve the amine but which are nonsolvents for and nondestructive of the substrate material. The solvent composition found to be suitable for use with the present compounds and for their application to transparencies produced therewith are hydrocarbon solvents such as hexane. Additionally, alcohols such as ethanol and isopropanol can be used. And further, mixtures of conventional solvents may be employed to attain the requisite coating on the transparency. Aside from the selection features mentioned above, the particular solvent utilized is not critical to the transparencies formed within the purview of the present invention. It is only necessary that the proper amounts of the coating compounds are dissolved in the aforementioned solvent mixture and that a continuous film is formed on evaporation of the solvent. Com-

pounds generally should be in a concentration of at least 0.3% by weight for optimum results.

It is, therefore, the selection of the particular amine materials which is critical for proper fixing and adhesion of the multicolored xerographic image to the transparency. It is also these materials which allow correct reproduction of color density in the fused image, as well as giving strength to the film which is needed for sheet transfer during copying and continuous use of the transparency after formation. The compounds used must also be compatible with the multi-component toners used for the subtractive color reproduction processes and accordingly prevent precipitation or deposition of the toner as discrete, recogniz-

able, particles in the final developed image as opposed to coalescence and formation of a uniform and consistent toner film. If the toner is deposited as recognizable and discrete particles, then an image is produced which has a "dirty" or spotty look and the color density thus becomes erratic. The coating materials must therefore be compatible with the toner materials used to develop the multicolor images, while at the same time being transparent and yet strong enough to permit normal handling of transparencies.

25 The amine compounds which may be used in the coating composition of the present invention may be any commercially available form of these materials. Suitable for use, for example, is 1,8-diamo octane, n-octadecyl amine, n-dodecyl amine, tallow amine, and 30 hydrogenated tallow amine all supplied by the Armour Industrial Chemical Company of Chicago, Ill.

The coating composition after dissolution in the appropriate solvent mixture is applied to the transparent thermoplastic film by techniques which are well known 35 to those skilled in the art of paper coating. Various techniques which are suitable for coating could be by roll, wire wound rod, air knife, or any other uniform application means used in paper coating. For instance, the coating may be simply passed (or dipped) through 40 a hopper containing the coating composition in liquid form, which is provided by a doctor blade or the coating may be applied by use of a more precise coating apparatus such as a gravure press. Preferably a coating of above about 0.1 mil thickness is produced upon the 45 transparent thermoplastic film sheet after evaporation of a solvent or solidification of the dissolved amine materials in the form of a film. Since the coating on the sheet is in the nature of an extremely thin film, no significant impairment of the transparency of the sheet 50 itself results from its presence and the transparency formed therefrom by electrostatic image evidences the requisite degree of clearness to be satisfactory for most visual education purposes.

55 The following represents a specific illustration of the present invention although it should be understood that the invention is not intended to be limited to specific details to be set forth thereon.

#### SPECIFIC EMBODIMENTS OF THE INVENTION

60 In the following illustrations two film types were used, LEXAN DL616 (a tetrachloro polycarbonate) and LEXAN SL1007 (a tetrabromo polycarbonate). The coatings on the transparencies were made by coating the films in the various solutions, air drying and curing at 150°-170°C. Prints were produced in a Xerox Model D processor (flat plate) using a premixed developer containing 10 g. of Xerox Cyan Toner, internally 65 designated as XT 1318C-13, and 500 g. of carrier ma-

terial, internally designated as XC910-20. Print fixing was accomplished in a Xerox Model D fuser which had temperatures ranging between 150°-170°C. The resulting transparencies were judged by projection using a "Telegraph-Resolute" mode 21105 overhead projector and rating on a transparency scale of from 1 to 10. Therefore, a rating of 1 indicates that no color whatsoever was visible on the projection screen while a rating of 10 indicates complete transparency.

Two materials, N-dodecylamine and N-octadecylamine, were analyzed in the aforementioned manner and appear in Table 1. The solvent used in all cases was hexane. Note that the transparency ratings of the particular coatings having requisite concentration have ratings of 7 or above which can be considered satisfactory and acceptable. Ratings of 5 are shown for those coating solutions in which the amount of amine falls below 0.3% by weight.

All of the coated transparent sheet materials are then subjected to a colored xerographic imaging process, as outlined above, with resultant heat fixing of the adherent image. It is observed that superior image adhesion occurred both before and after the fusion step. In addition, the colors reproduced are uniform, with consistent color density and with no evidence of toner "spotting". Additionally, the colored transparencies of the instant invention are found to exhibit lower frictional and static properties when compared with the uncoated transparencies.

It can be seen from the data set forth that the transparencies which are coated with the instant coating compounds exhibit improved toner adhesion properties and therefore are capable of better color image projection than those transparencies containing no coat.

There will now be obvious to those skilled in the art many modifications and variations of the invention set forth above. These modifications and variations will not, however, depart from the scope of the invention if defined by the following claims.

TABLE I

| Coating                     | Curing Time/Sec. | Print Fuse Time/Min. | Transparency |
|-----------------------------|------------------|----------------------|--------------|
| 0.3% h-dodecylamine/ hexane | 0                | 0.5                  | 7            |
| 0.3% h-dodecylamine/ hexane | 30               | 0.5                  | 7            |
| 0.3% h-dodecylamine/ hexane | 15               | 0.5                  | 10           |
| 0.3% h-dodecylamine/        |                  |                      |              |

TABLE I-continued

| Coating                        | Curing Time/Sec. | Print Fuse Time/Min. | Transparency |
|--------------------------------|------------------|----------------------|--------------|
| hexane                         | 5                | 0.5                  | 10           |
| 3% n-octadecyl amine/ hexane   | 60               | 1.0                  | 10           |
| 0.3% n-octadecyl amine/ hexane | 60               | 1.0                  | 10           |
| 0.1% n-octadecyl amine/ hexane | 60               | 1.0                  | 5            |
| 0.01% n-octadecyl amine/hexane | 60               | 1.0                  | 5            |
| 0.01% n-octadecyl amine hexane | 360              | 0.5                  | 5            |
| 0.3% n-octadecyl amine/ hexane | 360              | 0.5                  | 7            |

15 What is claimed is:

1. A method of xerographically preparing a color transparency copy comprising:

- forming a single color powder image of a multicolored original to be reproduced;
- transferring the powder image to a transparency comprising a thermoplastic film sheet, said sheet having at least one surface coated with a nonvolatile aliphatic amine, the amine coating having a thickness of above 0.1 mil; and
- fixing the powder image on the transparency.

20 2. The method of claim 1 wherein the steps of powder image formation and transfer are repeated before the fixing step, each sequence corresponding to the formation of a different color to effect multicolor reproduction, said transfer of each developed electrostatic image taking place in registration on the transparency.

25 3. The method of claim 1 wherein the fixing is carried out by heating.

30 4. The method of claim 1 wherein the transparency used in the transfer step is a thermoplastic film sheet of polysulfone, polycarbonate, or polyester material.

35 5. The method of claim 1 wherein the step of forming a single color powder image comprises:

- exposing a charged photoconductive member to a filtered light image of the multicolored original to record a single color electrostatic latent image thereon; and
- developing the single color electrostatic latent image with toner particles complementary in color thereto.

40 45 6. The method of claim 1 wherein said amine is selected from the group consisting of 1,8-diamino octane, n-octadecyl amine, n-dodecyl amine and mixtures thereof.

\* \* \* \* \*